

Jan. 9, 1968

W. R. BARBER, JR.

3,362,812

ALLOY STEEL AND METHOD

Filed July 6, 1965

PHYSICAL PROPERTIES  
OF VANDIUM ALLOY STEELS WITH & WITHOUT CHROMIUM



----- = ABOUT 0.32 Cr.

— = ABOUT 1.50 Cr.

INVENTOR:

WILLIAM R. BARBER, JR.

BY

*Dawson, Tilton, Fallon, Lungmug & Alexander*  
ATT'YS

# United States Patent Office

3,362,812

Patented Jan. 9, 1968

1

3,362,812

## ALLOY STEEL AND METHOD

William R. Barber, Jr., Portland, Oreg., assignor to Esco Corporation, Portland, Oreg., a corporation of Oregon  
Filed July 6, 1965, Ser. No. 469,577  
7 Claims. (Cl. 75—126)

This invention relates to an alloy steel and method of preparation and, more particularly, to a modified Hadfield's steel useful in abrasive operations.

Hadfield's steel became known early in this century (see U.S. Patent 856,250). It is generally regarded as an austenitic manganese steel (carbon about 1%, manganese 10–14%) which, although soft in the heated treated condition, becomes surface-hardened through cold working. This develops a particular wear life and over the years many attempts have been made to improve the wear life by adding various alloying materials.

I have found that wear life of austenitic manganese steel can be materially extended by adding specific amounts of vanadium and chromium to Hadfield's steel, and this without the need for exotic heat treatments deemed necessary in the past as art workers attempted to improve the physical characteristics of Hadfield's steel. The provision of this new alloy, the method of preparing the same, and the method of developing various useful products therewith constitute important objectives of the invention. Other objects may be seen in the subsequent details of this specification.

The invention is explained in conjunction with the accompanying drawing which is a chart of various physical characteristics as a function of vanadium content of high and low chromium Hadfield steels.

2

heated to 2000° F., for two hours after which the temperature was dropped to 1750° F., for one-half hour and thereafter water quenched. Jaws produced according to this procedure had wear lives well in excess of jaws similarly prepared, but without vanadium. On one application of jaws for the above-mentioned 10" × 36" Cedar Rapids crushed operated in a Western quarry, the life was increased from a normal output of 6000 tons to 18,000 tons.

Further investigation revealed that when using good heat treating procedures for manganese steels (both with and without chromium) very few undissolved carbides can be observed in the grain boundaries or in the matrix of the steel. However, even when as little as 0.25% vanadium is added, a pronounced carbide appears in the austenitic matrix (in the form of small spots when microscopically observed at 100×). Still further, as the percent of vanadium is increased, so also does the number of spots. From this, I believe that the combination of chromium and vanadium suppresses the formation of the carbide by promoting a more uniform scattering of the carbide in the matrix with the consequent development of a harder matrix.

Other field tests show that the chromium vanadium alloy provides greater service life than a regular austenitic manganese steel containing vanadium only, i.e., without chromium.

To ascertain the optimum ranges of alloy materials, a series of test bars were made according to the procedure of the example, i.e., quenching from above 1700° F., and tested for various physical characteristics, the formulations and results being tabulated in Table II. From these results, the charts of the drawing were made:

TABLE II

|                    | Chromium | Silicon | Manganese | Vanadium | Carbon | Tens. Str., p.s.i. | Yld. Str., p.s.i. | Elong., in 2", percent | Red. of Area, percent | Hardness, BHN | Charpy V-Notch, ft.-lbs. | Avg. |
|--------------------|----------|---------|-----------|----------|--------|--------------------|-------------------|------------------------|-----------------------|---------------|--------------------------|------|
| No. E*             | 1.50     | 0.38    | 12.85     | 0.98     | 1.30   | 113,000            | 68,250            | 17                     | 17                    | 241           | 13-15                    | 14   |
| No. 1              | 1.65     | 0.54    | 12.35     | 1.38     | 1.12   | 115,000            | 64,700            | 14                     | 13                    | 255           | 9-9½                     | 9    |
| No. 2              | 0.32     | 0.45    | 12.95     | 1.14     | 1.11   | 99,750             | 57,250            | 14                     | 13                    | 235           | 14½-11½                  | 13   |
| No. 3              | 1.60     | 0.55    | 12.65     | 1.14     | 1.18   | 110,600            | 65,700            | 14                     | 14                    | 241           | 10½-8½                   | 9½   |
| No. 4              | 0.32     | 0.45    | 12.95     | 1.14     | 1.12   | 107,750            | 58,500            | 16                     | 15                    | 235           | 15½-17                   | 16   |
| No. 5              | 1.60     | 0.53    | 12.85     | 0.64     | 1.22   | 118,750            | 67,500            | 25                     | 24                    | 229           | 38½-28                   | 33   |
| No. 6              | 0.32     | 0.45    | 12.95     | 0.64     | 1.14   | 117,250            | 58,500            | 29                     | 27                    | 217           | 62-63½                   | 63   |
| No. 7              | 1.75     | 0.53    | 12.85     | 0.37     | 1.24   | 103,000            | 64,900            | 22                     | 20                    | 229           | 25½-27                   | 26   |
| No. 8              | 0.32     | 0.45    | 12.95     | 0.37     | 1.14   | 125,750            | 55,500            | 43                     | 32                    | 217           | 90-72                    | 81   |
| No. 9              | 1.85     | 0.54    | 12.95     | 0.17     | 1.24   | 98,000             | 65,400            | 22                     | 22                    | 212           | 31½-35½                  | 33½  |
| No. 10             | 0.32     | 0.45    | 12.95     | 0.17     | 1.16   | 124,750            | 54,000            | 53                     | 40                    | 207           | 145-149½                 | 147  |
| No. 11 (Hadfields) | 0.32     | 0.45    | 12.95     | -----    | 1.10   | 116,000            | 48,000            | 52                     | 37                    | 201           | 192½-231                 | 212  |
| No. 12             | 1.50     | 0.38    | 12.85     | -----    | 1.30   | 122,500            | 62,000            | 35                     | 32                    | 212           | 44                       | 44   |

\*This is the formulation of the example.

The invention can be best appreciated from a specific example which demonstrated the substantial improvement in wear life achieved through the practice of the invention.

### Example

For casting jaws for a 10" × 36" Cedar Rapids crusher, the following formulation was employed.

TABLE I

|                                    | Percent |
|------------------------------------|---------|
| Chromium                           | 1.50    |
| Silicon                            | 0.38    |
| Manganese                          | 12.85   |
| Vanadium                           | 0.98    |
| Carbon                             | 1.30    |
| Iron (usual impurities) Remainder. |         |

The casting procedure included adding the vanadium in the form of Carvan, a high carbon ferrovanadium marketed by Union Carbide. After casting, the jaws were

The pattern followed in making the runs 1–10 was to compare a chromium vanadium alloy (runs 1, 3, 5, 7, and 9) with a vanadium alloy (runs 2, 4, 6, 8, and 10) of the same "target" composition. For example in runs 1 and 2, it was intended to have 1.50% vanadium (based upon the amount of vanadium added to the melt) with run 1 including additionally 1.50% chromium. Thus, in each of runs 1, 3, 5, 7, and 9 the target was 1.50% chromium, but this was not precisely attained due to the impossibility of accounting for the presence of unintended impurities. Likewise, in runs 2, 4, 6, 8 and 10, it was intended to have no chromium. The analyses subsequent to casting are those reported. Further, in the various runs, the amount of vanadium was decreased, i.e., for runs 1 and 2 a target of 1.50%, for runs 3 and 4 a target of 1.25%, for runs 5 and 6 a target of 1.00%, for runs 7 and 8 a target of 0.50%, and for runs 9 and 10 a target of 0.25% vanadium. Runs E and 12 correspond to the formulations used in the 18,000 lb. and 6000 lb. life jaws, respectively.

Plotting of the various physical characteristics reveals an unexpected "peaking" in the range of 0.60-1.05% vanadium when chromium is present and all of the curves demonstrate a pronounced improvement in the various physical characteristics when the particular curve for vanadium alloys with chromium is compared with the corresponding curve for the same alloy without chromium.

Table III below summarizes my findings on the useful ranges of alloy constituents:

TABLE III

| Ingredient     | Useful    | Optimum   | Target   |
|----------------|-----------|-----------|----------|
| Chromium.....  | 1.0-2.0   | 1.3-1.6   | 1.5      |
| Silicon.....   | 0.15-0.70 | 0.40-0.60 | 0.50     |
| Manganese..... | 10.5-14.0 | 11.5-13.5 | 12.5     |
| Vanadium.....  | .25-1.5   | .60-1.05  | .60-1.05 |
| Carbon.....    | 0.90-1.40 | 1.20-1.35 | 1.25     |

The vanadium target is set dependent upon the combination of physical characteristics sought, it being appreciated that the remainder is iron with the usual impurities associated therewith. In this connection, I prefer to maintain sulfur and phosphorus each below a maximum of 0.04%.

Relative to the amount of vanadium employed, I find useful percentages in the range of 0.60-0.80% where the casting is relatively unsupported as in the case of a crusher bowl liner. However, where ductility can be sacrificed in favor of increased wear life, as in a supported crusher jaw, the vanadium is set at the high end of the optimum range and may advantageously go to 1.25% for certain crusher jaws.

Using 0.98% vanadium in a hammermill installation resulted in an increase of 170 tons wear life (using Run 12 alloy) to 202 tons (using Run E alloy) before replacement was necessary.

In summary I have observed the following:

(1) Vanadium added in the amounts from .25-1.25% to an 11-14% austenitic manganese steel, with approximately 1.50% chromium, will give increased hardness to the alloy when the alloy is quenched in water in the normal manner for manganese alloys from a temperature greater than 1700° F.

(2) The preferred addition of vanadium to the base analysis of the chromium-bearing austenitic manganese steel is about .60-.80% since this provides the best combination of mechanical properties. However, if ductility can be sacrificed for potential increased wear, then the vanadium may be increased to a value as high as 1.25%.

(3) The hardness, BHN, will increase as the vanadium content of the base alloy is increased from .25-1.25%. This increased hardness of the metal over the base alloy undoubtedly minimizes the initial wear on a part before the usual work hardening occurs.

(4) When the vanadium content is increased above .20% the yield strength of the alloy increases drastically from about 55,000 p.s.i. to about 70,000 p.s.i. This increase in yield strength is also quite helpful in preventing the metal from flowing or spreading out, which usu-

ally happens with the regular 11-14% austenitic manganese alloy.

While in the foregoing specification, a detailed description of the invention has been set down for the purpose of illustration, many variations in the details herein given may be made by those skilled in the art without departing from the spirit and scope of the invention.

I claim:

1. An austenitic manganese steel useful in abrasive applications consisting essentially of from about 1.0% to about 2.0% chromium, from about 0.15% to about 0.70% silicon, from about 10.5% to about 14.5% manganese, from about 0.25% to about 1.5% vanadium, from about 0.90% to about 1.40% carbon with the balance iron including the usual impurities associated therewith, with a maximum of about 0.04% each of phosphorus and sulphur.

2. An austenitic manganese steel useful in abrasive applications consisting essentially of from about 1.3% to about 1.6% chromium, from about 0.040% to about 0.60% silicon, from about 11.5% to about 13.5% manganese, from about 0.60% to about 1.50% vanadium, from about 1.20% to about 1.35% carbon with the balance iron including the usual impurities associated therewith, with a maximum of about 0.04% each of phosphorus with sulphur.

3. The steel of claim 2 in which the chromium is about 1.5%, the silicon 0.50%, the manganese about 12.5% and the carbon 1.25%.

4. A method of preparing an abrasion resistant alloy steel comprising casting a mixture of from about 1.3% to about 1.6% chromium, from 0.40% to about 0.60% silicon, from about 11.5% to about 13.5% manganese, from about 1.20% to about 1.35% carbon and an amount of vanadium in the range of about 0.60% to about 1.05% along with iron and water quenching the casting from above about 1700° F., the amount of vanadium employed being in the lower end of the above-mentioned range when the casting is employed in an environment where self-support is needed and being in the higher end of the range where the casting is substantially supported in operation.

5. The method of claim 4 in which said casting is a crusher jaw.

6. The method of claim 4 in which said casting is a bowl liner.

7. The method of claim 4 in which said casting is a crusher hammer.

#### References Cited

##### UNITED STATES PATENTS

|           |         |              |       |          |
|-----------|---------|--------------|-------|----------|
| 436,497   | 9/1890  | Hadfield     | ----- | 75-126   |
| 1,310,528 | 7/1919  | Hadfield     | ----- | 75-126   |
| 1,435,294 | 11/1922 | Hadfield     | ----- | 75-126   |
| 2,382,651 | 8/1945  | Nesbitt      | ----- | 75-126 X |
| 2,865,740 | 12/1958 | Heger et al. | ----- | 75-123   |

DAVID L. RECK, Primary Examiner.

P. WEINSTEIN, Assistant Examiner.